

## UNITED STATES PATENT OFFICE

2,637,667

PROCESS FOR PREPARING STEELS AND  
ALLOYS FOR ROLLINGWilliam Oakley Binder, Niagara Falls, N. Y., as  
signor to Union Carbide and Carbon Corpora-  
tion, a corporation of New YorkNo Drawing. Application January 8, 1952,  
Serial No. 265,545

12 Claims. (Cl. 134—4)

1

This invention relates to a method for removing surface imperfections from steels and alloys and is particularly useful for treating the surfaces of these materials prior to a shaping operation such as rolling.

Ingots, slabs, billets, castings and the like usually have surfaces that are unsuitable in finished articles. If the metal is to be rolled, some of the surface imperfections are eliminated during normal rolling, but others are so serious that they detrimentally affect the quality of the finished article unless they are removed before the final rolling. The more objectionable surface imperfections are attributable, for example, to seams, scabs, and blowholes. Conventionally, these more objectionable imperfections are removed by such operations as grinding and chipping the metal, both of which are tedious, laborious and wasteful operations. Castings also often have undesirable surface imperfections and these too are eliminated conventionally by removing part of the metal of the casting by grinding, chipping or the like.

It is an object of the invention to provide a method for removing imperfections from the surfaces of bodies of steel or other alloys.

Another object of the invention is to provide a method for eliminating defects in the surfaces of semifinished articles of steel and other alloys which defects can impair finished products rolled from the semifinished articles.

The objects of the invention are accomplished by heating an article of steel or alloy to a temperature of between 700° C. and 1200° C. and exposing the article while it is in that temperature range to a gaseous sulfur compound as described below. Best results have been obtained with treatments at temperatures of from 950° C. to 1050° C. During this treatment the metal is attacked generally and a loose scale forms on its surface. This scale can be easily removed, for example by chipping or sandblasting, the work being required to remove this loose scale being much less than that required for chipping or sandblasting the metal itself. Under the scale is a smooth surface relatively free of imperfections. If the treatment is continued long enough, the injurious and undesirable imperfections on the surface are eliminated.

The sulfur compounds used in the process must be those which are normally gaseous at a temperature of between 700° C. and 1200° C., and preferably at a temperature of about 700° C. They must also be ones which will dissociate at a temperature of between 700° C. and 1200° C. in the presence of the steel or alloy being treated

2

to make sulfur available for reaction with the steel or alloy. Sulfur containing compounds which dissociate to free oxygen should be avoided since oxygen tends to attack the metals intergranularly rather than generally. The preferred compound is hydrogen sulfide. Examples of other compounds that can be used are sulfur dichloride, sulfur tetrachloride, ammonium sulfide, and carbon bisulfide. With some of these compounds certain incidental effects such as mild carburizing and nitriding are obtained.

It has been found that when certain alloys are treated at temperatures above about 850° C. for times sufficient to remove relatively deep surface imperfections, two scales are formed. For example, when surface imperfections are removed according to the invention from alloys containing nickel, cobalt and more than about 18% chromium by holding these materials at about 1000° C. in a stream of hydrogen sulfide, an inner scale 15 may be formed in addition to the loose scale mentioned above. This inner scale is thin and adheres tightly to the treated metal so that it cannot be removed as readily by sandblasting and chipping as the loose outer scale. This inner scale 20 may detrimentally affect the treated metal if it is not removed. For example, if the metal is to be rolled further, the inner scale tends to penetrate the metal intergranularly and cause shallow surface cracking. The inner scale also 25 tends to diminish the resistance of the metal to corrosive attack.

The inner scale may be removed by again treating the metal with the gaseous sulfur compound, in this instance hydrogen sulfide, at a temperature of from 700° C. to 850° C. A temperature of 35 800° C. is preferred for this treatment. In general, an exposure of the metal for one hour to the gas at the preferred temperature will loosen the inner scale so that it can be removed readily by 40 sandblasting or otherwise.

The method of the invention has been found to be satisfactory for the treatment of a great number of steels and alloys. Among those to which the method has been successfully applied 45 are: Carbon steels, chromium steels having from 5% to 25% chromium, 18/8 stainless steel, stainless steel containing titanium or columbium, nickel-base chromium-iron alloys, and chromium-cobalt-tungsten alloys. Excellent results 50 have been obtained with the steels and other alloys containing chromium. If more than about 10% molybdenum is present in the alloy, the scale formed is often difficult to remove. For this reason, best results with molybdenum containing 55 alloys have been obtained with those alloys

having a molybdenum content of less than about 10%.

The rate at which the metal is attacked and the imperfections eliminated depends upon the temperature, composition of the metal being treated, and the thickness of the scale layer present as a result of the treatment. For example, with alloys containing up to 25% chromium, an exposure to hydrogen sulfide at 1000° C. for a period of eight hours will result in the removal of from 0.05 to 0.075 of an inch of metal. At 900° C. and an exposure of two hours to hydrogen sulfide, the same materials will lose from 0.005 to 0.012 of an inch of metal. In two hours at 1000° C. these same materials will lose from 0.019 to 0.027 of an inch of metal, and at 1100° C. with the same time of treatment the loss of metal is from 0.031 to 0.036 of an inch.

The removal of metal can be hastened by periodically removing the loose scale formed. For example, if an alloy similar to the one described above is exposed to the hydrogen sulfide for two one-hour periods at 1000° C. and the scale is removed after the first exposure, the total metal removed is from 0.028 to 0.035 of an inch as compared with 0.019 to 0.027 of an inch if the exposure is for two continuous hours.

The exact time that the alloy is exposed to the gaseous sulfur compound will depend upon the requirements in particular instances. As has been shown above an increase in temperature will in general result in the more rapid removal of metal. However, at temperatures of about 1100° C. and above there is a tendency for the scale to fuse which slows down the action of the sulfur and renders the scale more difficult to remove.

What is claimed is:

1. A process for eliminating surface imperfections from metal which comprises exposing said metal to an atmosphere of a gaseous sulfur compound at a temperature of from 700° C. to 1200° C., effecting the dissociation of the compound to provide sulfur to combine with said metal, maintaining said metal at a temperature of from 700° C. to 1200° C., and subsequently removing from said metal a scale formed on the surface of said metal during said exposure to said gaseous sulfur compound.

2. A process for eliminating surface imperfections from metal which comprises exposing said metal to an atmosphere of a gaseous sulfur compound at a temperature of from 950° C. to 1050° C., effecting the dissociation of the compound to provide sulfur to combine with said metal, maintaining said metal at a temperature of from 950° C. to 1050° C., and subsequently removing from said metal a scale formed on the surface of said metal during said exposure to said gaseous sulfur compound.

3. A process for eliminating surface imperfections from a chromium containing alloy, which process comprises exposing said alloy to an atmosphere of a gaseous sulfur compound at a temperature of from 850° C. to 1200° C., effecting the dissociation of the compound to provide sulfur to combine with said metal, maintaining said alloy at a temperature of from 850° C. to 1200° C. to form a loose outer scale and an adherent inner scale on said alloy, removing from said alloy the loose outer scale, exposing said alloy with said adherent scale to an atmosphere of a gaseous sulfur compound at a temperature of from 700° C. to 850° C., effecting the dissociation of the compound to provide sulfur to combine with said metal, maintaining said alloy at a temperature of

from 700° C. to 850° C. to convert said adherent scale to a loose scale, and removing the latter said loose scale.

4. A process for eliminating surface imperfections from a chromium containing alloy, which process comprises exposing said alloy to an atmosphere of a gaseous sulfur compound at a temperature of from 950° C. to 1050° C., effecting the dissociation of the compound to provide sulfur to combine with said metal, maintaining said alloy at a temperature of from 950° C. to 1050° C. to form a loose outer scale and an adherent inner scale on said alloy, removing from said alloy the loose outer scale, exposing said alloy with said adherent scale to an atmosphere of a gaseous sulfur compound at a temperature of about 800° C., effecting the dissociation of the compound to provide sulfur to combine with said metal, maintaining said alloy at a temperature of about 800° C. to convert said adherent scale to a loose scale, and removing the latter said loose scale.

5. A process for eliminating surface imperfections from metal which comprises exposing said metal to an atmosphere of hydrogen sulfide while maintaining said metal at a temperature of from 700° C. to 1200° C., and subsequently removing from said metal a scale formed on the surface of said metal during said exposure to an atmosphere of hydrogen sulfide.

6. A process according to claim 5 wherein said metal is steel.

7. A process according to claim 5 wherein said metal is an alloy containing chromium.

8. A process for eliminating surface imperfections from metal which comprises exposing said metal to an atmosphere of hydrogen sulfide while maintaining said metal at a temperature of from 950° C. to 1050° C., and subsequently removing from said metal a scale formed on the surface of said metal during said exposure to an atmosphere of hydrogen sulfide.

9. A process according to claim 8 wherein said metal is steel.

10. A process according to claim 8 wherein said metal is an alloy containing chromium.

11. A process for eliminating surface imperfections from a chromium containing alloy which process comprises exposing said alloy to an atmosphere of hydrogen sulfide while maintaining said alloy at a temperature of from 850° C. to 1200° C. to form a loose outer scale and an adherent inner scale on said alloy, removing from said alloy the loose outer scale, exposing said alloy with said adherent scale to an atmosphere of hydrogen sulfide while maintaining said alloy at a temperature of from 700° C. to 850° C. to convert said adherent scale to a loose scale, and removing the latter said loose scale.

12. A process for eliminating surface imperfections from a chromium containing alloy which process comprises exposing said alloy to an atmosphere of hydrogen sulfide while maintaining said alloy at a temperature of from 950° C. to 1050° C. to form a loose outer scale and an adherent inner scale on said alloy, removing from said alloy the loose outer scale, exposing said alloy with said adherent scale to an atmosphere of hydrogen sulfide while maintaining said alloy at a temperature of about 800° C. to convert said adherent scale to a loose scale, and removing the latter said loose scale.

WILLIAM OAKLEY BINDER.

No references cited.